



US005376208A

**United States Patent [19]****Yao et al.****[11] Patent Number: 5,376,208****[45] Date of Patent: Dec. 27, 1994****[54] WATER-PERMEABLE AND FIRE-RESISTANT PRODUCT AND A PREPARING METHOD THEREOF**

**[75] Inventors:** **Shin-Chuan Yao, Tu Cheng, Jong-Fu Wu, Kun-Lin Cheng**, both of Taipei; **Chiu-Hsiung Tsai, Yun Lin Hsien; Farn-Ping Koong**, Taipei; **Kun-Lung Chuang, Tao Yuan Hsien; Shu-Lan Yao, Yung Ho; Chin-Liu Liu, Chuang**, all of Taiwan, Prov. of China

**[73] Assignee:** **China Textile Institute, Tu Cheng, Taiwan, Prov. of China**

**[21] Appl. No.:** **241,406**

**[22] Filed:** **May 11, 1994**

**[51] Int. Cl.<sup>5</sup>** ..... **B29C 47/00; B32B 5/18**

**[52] U.S. Cl.** ..... **156/246; 156/78; 428/260; 428/317.1; 428/318.4; 428/921; 521/88; 521/91; 521/92; 521/98; 521/64; 521/114; 521/124; 521/125; 521/132; 521/906; 524/371; 524/411; 524/412**

**[58] Field of Search** ..... **156/78, 246; 428/260, 428/317.1, 318.4; 521/88, 92, 906, 64, 91, 98, 114, 124, 125, 132; 524/371, 411, 412**

**[56]****References Cited****U.S. PATENT DOCUMENTS**

4,836,875 6/1989 Buttermore et al. ..... 156/246  
5,035,763 7/1991 Wegner et al. ..... 156/246  
5,114,515 5/1992 Birdwell et al. ..... 156/246

*Primary Examiner*—Morton Foelak

*Attorney, Agent, or Firm*—Morton J. Rosenberg; David I. Klein

**[57]****ABSTRACT**

A water-permeable and fire-resistant product and the preparing method thereof is disclosed. The water-permeable and fire-resistant product is made of a fabric layer and a porous film adhered thereon. The porous film of this invention comprises polyurethane resin; a first fire-resistant agent; a second fire-resistant agent, an inorganic fire-resistant agent and an additive agent. The first fire-resistant agent used is selected from the group consisting of paraffine chlorinated, decabromodiphenyl oxide, hexachloro benzene, hexabromo benzene, pentabromo ethyl benzene, pentabromo diphenyl oxide and octabromo diphenyl ether. The second fire-resistant agent used is selected from the group consisting of Sb<sub>2</sub>O<sub>3</sub> and Sb<sub>2</sub>O<sub>5</sub>. The surface of the product produced is smooth.

**6 Claims, No Drawings**

**WATER-PERMEABLE AND FIRE-RESISTANT  
PRODUCT AND A PREPARING METHOD  
THEREOF**

**FIELD OF THE INVENTION**

This invention relates to a water-permeable and fire-resistant product and the preparing method thereof. In particular, this invention relates to a product with a smooth surface.

**BACKGROUND OF THE INVENTION**

Polyurethanes are widely known as cushions, pillows, sofa, suitcase, soundproof material. Since polyurethanes do not provide heat-resistant property, the users mix polyurethanes with halogen-included compound, phosphoric compound, organic compound or inorganic compound to increase the fire-resistant effect thereof. However, all of fire-resistant agents used are water soluble and will dissolve in water. Therefore, the product produced lacks the fire-resistant property.

**SUMMARY OF THE INVENTION**

The object of this invention is to provide a water-permeable and fire-resistant product which has a smooth surface.

The other object of this invention is to provide a water-permeable and fire-resistant product which can eliminate the disadvantages of the prior art and easily prepared.

**DETAILED DESCRIPTION OF THE  
PREFERRED EMBODIMENT**

The water-permeable and fire-resistant product of this invention is made of a fabric layer and a porous film. The porous film is comprises polyurethane resin; a first fire-resistant agent; a second fire-resistant agent, an inorganic fire-resistant agent and an additive agent. The first fire-resistant agent used is selected from the group consisting of paraffins chlorinated, decabromodiphenyl oxide, hexachloro benzene, hexabromo benzene, pentabromo ethyl benzene, pentabromo diphenyl oxide and octabromo diphenyl ether. The second fire-resistant agent selected from the group consisting of Sb<sub>2</sub>O<sub>3</sub> and Sb<sub>2</sub>O<sub>5</sub>. The weight ratio between the first fire-resistant agent and the second fire-resistant agent is from 1:10 to 10:1. The weight ratio between the first fire-resistant agent and the second fire-resistant agent is from 1:1 to 4:1. The inorganic fire-resistant agent is selected from the group consisting of Mg(OH)<sub>2</sub>, MoO<sub>3</sub>, Al(OH)<sub>3</sub>, P, CaCO<sub>3</sub>, CaOAl<sub>2</sub>O<sub>3</sub>.6H<sub>2</sub>O, MgCO<sub>3</sub>, CuO and Cu<sub>2</sub>O. The additive agent is selected from the group consisting of Zn, Mg, ZrO<sub>2</sub>, TiO<sub>2</sub>, SiO<sub>2</sub>, SnO, ZnO and BaB<sub>2</sub>O<sub>4</sub>. The amount of the inorganic fire-resistant agent based on the weight of the polyurethane resin is from 5 to 100 wt%. The amount of said additive agent based on the weight of the polyurethane resin is from 2 to 30 wt%.

The present method for preparing water-permeable and fire-resistant product comprises the steps of (a) mixing polyurethane resin with a first fire-resistant agent selected from the group consisting of paraffin chlorinated, decabromodiphenyl oxide, hexachloro benzene, hexabromo benzene, pentabromo ethyl benzene, pentabromo diphenyl oxide and octabromo diphenyl ether; a second fire-resistant agent selected from the group consisting of Sb<sub>2</sub>O<sub>3</sub> and Sb<sub>2</sub>O<sub>5</sub>; an inorganic fire-resistant agent and an additive agent to form a mixture; (b) grinding said mixture; (c) formulating said

mixture to form a coating solution; (d) applying said coated solution to a support; (e) wet-curing said coated solution applied on said support to form a film and (f) adhering said film on a fabric layer. The weight ratio between the first fire-resistant agent and the second fire-resistant agent is from 1:10 to 10:1. The weight ratio between the first fire-resistant agent and the second fire-resistant agent is from 1:1 to 4:1. The inorganic fire-resistant agent is selected from the group consisting of Mg(OH)<sub>2</sub>, MoO<sub>3</sub>, Al(OH)<sub>3</sub>, P, CaCO<sub>3</sub>, CaOAl<sub>2</sub>O<sub>3</sub>.6H<sub>2</sub>O, MgCO<sub>3</sub>, CuO and Cu<sub>2</sub>O. The additive agent is selected from the group consisting of Zn, Mg, ZrO<sub>2</sub>, TiO<sub>2</sub>, SiO<sub>2</sub>, SnO, ZnO and BaB<sub>2</sub>O<sub>4</sub>. The amount of the inorganic fire-resistant agent based on the weight of the polyurethane resin is from 5 to 100 wt%. The amount of said additive agent based on the weight of the polyurethane resin is from 2 to 30 wt %. The wet-curing process of the present method is carried out at a temperature of from 10 to 50°J for 0.5 to 20 minutes.

The present invention will now be described more specifically with reference to the following preferred embodiment. It is to be noted that the following descriptions of the preferred embodiment of this invention are presented herein for the purpose of illustration and description; it is not intended to be exhaustive or to limit the invention to the precise form disclosed.

**EXAMPLE 1**

30 The amount of polyurethane and the fire-resistant agents are respectively listed in Table 1.

The reactants listed in Table 1 can be mixed to form a coating solution.

35 The solution is applied on a support with an amount of 300 g/m<sup>2</sup> and was wet-cured at a temperature of 20°J for 10 minutes. After water-washing, the cured-product was drying at a temperature of 140 °J. The resulted product was tested according ASTM 2863 -74 and LYSSY method at a temperature 40°J and 95% RH. The results of the test are described in Table 1.

**EXAMPLES 2-3 AND COMPARED EXAMPLES  
1-2**

45 The preparing process of these examples were the same as that of EXAMPLE 1 and the reactants used also listed in Table 1. The resulted products of these examples are also described in Table 2.

Viewing the results listed in Table 2, the L.O.I. values of the Examples 1 to 3 are better than that of Compared Example 1 and 2.

**TABLE 1**

| RE-ACTANTS                     | EXAMPLE    |            |            |                      |                      |
|--------------------------------|------------|------------|------------|----------------------|----------------------|
|                                | EX-AMPLE 1 | EX-AMPLE 2 | EX-AMPLE 3 | COM-PARED EX-AMPLE 1 | COM-PARED EX-AMPLE 2 |
| polyurethane                   | 100 g      | 100 g      | 100 g      | 100 g                | 100 g                |
| paraffine chlorinated          | 20 g       | 25 g       | 22.5 g     | 20 g                 | 0 g                  |
| Sb <sub>2</sub> O <sub>5</sub> | 5 g        | 10 g       | 7.5 g      | 10 g                 | 0 g                  |
| Mg(OH) <sub>2</sub>            | 10 g       | 10 g       | 10 g       | 0 g                  | 0 g                  |
| Al(OH) <sub>3</sub>            | 10 g       | 10 g       | 0 g        | 0 g                  | 0 g                  |
| MoO <sub>3</sub>               | 10 g       | 0 g        | 0 g        | 0 g                  | 0 g                  |
| ZnO                            | 15 g       | 15 g       | 15 g       | 0 g                  | 0 g                  |
| ZrO <sub>2</sub>               | 0 g        | 0 g        | 10 g       | 0 g                  | 0 g                  |
| anion surfactant               | 2 g        | 2 g        | 2 g        | 2 g                  | 2 g                  |

TABLE 1-continued

| RE-ACTANTS | EXAMPLE    |            |            | COM-PARED  | COM-PARED  |
|------------|------------|------------|------------|------------|------------|
|            | EX-AMPLE 1 | EX-AMPLE 2 | EX-AMPLE 3 | EX-AMPLE 1 | EX-AMPLE 2 |
| pigment    | 20 g       | 10 g       | 10 g       | 10 g       | 20 g       |

TABLE 2

| PROPERTIES<br>EXAMPLE | L.O.I. | WATER-PERMEABLE<br>PROPERTIES |  | SOFTNESS  |
|-----------------------|--------|-------------------------------|--|-----------|
|                       |        |                               |  |           |
| EXAMPLE 1             | 43     | 9500                          |  | EXCELLENT |
| EXAMPLE 2             | 41     | 9000                          |  | EXCELLENT |
| EXAMPLE 3             | 38     | 9000                          |  | EXCELLENT |
| COMPARED              | 28     | 5000                          |  | GOOD      |
| EXAMPLE 1<br>COMPARED | 24     | 4500                          |  | FAIL      |
| EXAMPLE 2             |        |                               |  |           |

We claim:

1. A method for preparing water-permeable and fire-resistant product comprising the steps of:

mixing polyurethane resin with a first fire-resistant agent selected from the group consisting of paraffin chlorinated, decabromodiphenyl oxide, hexachloro benzene, hexabromo benzene, pentabromo ethyl benzene, pentabromo diphenyl oxide and octabromo diphenyl ether; a second fire-resistant agent is selected from the group consisting of Mg(OH)<sub>2</sub>, MoO<sub>3</sub>, Al(OH)<sub>3</sub>, P, CaCO<sub>3</sub>, CaAl<sub>2</sub>O<sub>3</sub>.6H<sub>2</sub>O, MgCo<sub>3</sub>, CuO and Cu<sub>2</sub>O selected from the group

consisting of Sb<sub>2</sub>O<sub>3</sub> and Sb<sub>2</sub>O<sub>5</sub>; an inorganic fire-resistant agent is selected from the group consisting of Zn, Mg, ZrO<sub>2</sub>, TiO<sub>2</sub>, SiO<sub>2</sub>, SnO, ZnO and an additive agent to form a mixture;

5 grinding said mixture; formulating said mixture to form a coating solution; applying said coating solution to a support; wet-curing said coating solution on said support to form a film; and adhering said film on a fabric layer.

10 2. A method for preparing water-permeable and fire-resistant product as claimed in claim 1, wherein the weight ratio between said first fire-resistant agent and said second fire-resistant agent is from 1:10 to 10:1.

15 3. A method for preparing water-permeable and fire-resistant product as claimed in claim 1, wherein the weight ratio between said first fire-resistant agent and said second fire-resistant agent is from 1:1 to 4:1.

20 4. A method for preparing water-permeable and fire-resistant product as claimed in claim 1, wherein the amount of said inorganic fire-resistant agent based on the weight of said polyurethane resin is from 5 to 100 wt%.

5. A method for preparing water-permeable and fire-resistant product as claimed in claim 1, wherein the amount of said additive agent based on the weight of said polyurethane resin is from 2 to 30 wt%.

25 6. A method for preparing water-permeable and fire-resistant product as claimed in claim 1, wherein said wet-curing process is carried out at a temperature of from 10 to 50°J for 0.5 to 20 minutes.

\* \* \* \* \*